

# United States Patent Office

**2,868,665**

Patented Jan. 13, 1959

1

2,868,665

**AN IMPREGNATED CORRUGATED PAPERBOARD,  
A COMPOSITION THEREFOR, AND A PROCESS  
OF MAKING SAID COMPOSITION**

Albert R. McManus, St. Louis, Mo.

**No Drawing. Application March 7, 1957**  
**Serial No. 644,476**

**6 Claims. (Cl. 106—230)**

The invention relates to a new and useful impregnant for paperboard which increases the column loading strength to at least about 300 percent, and beam loading strength at least 200 percent regardless of humidity conditions.

The present invention comprises fully refined 133° F. melting point paraffin and limed rosin having about 4.5 percent lime content in the ratio of from 45 : 55 to 55 : 45 respectively. The said mixture is prepared by charging substantially equal quantities by weight into a suitable vessel and heating to 325° F. with some occasional mild agitation. I have found that 180 p. s. i. steam in coils a safe and desirable method of melting the mixture and holding it at about 325° F.

In recent years there has been an increasing demand for an inexpensive strength imparting and water resistant paperboard impregnant to be used for fruit and vegetable containers which, in the field are subjected to high humidity conditions, and containers that are stacked many times out in warehouses for long periods of time.

Ordinarily the entire container is not impregnated as the surface of the impregnated paperboard is unsatisfactory for printing, etc. Therefore, impregnated liners or corner posts are placed inside the container to provide the increased top load strength required.

I have found that corrugated paperboard is most easily

2

compositon do not materially stiffen the corrugated paper-board, but only add to the cost. Optimum stiffening per quantity of impregnating compositon used therefore is obtained by impregnating the impregnating composition into paperboard and filling all interstices between the fibers and not merely coating the surface thereof. To do this, the impregnating composition must be highly fluid at the application temperature and of a nature to be absorbed into and cling tightly to the fibres and to fill all voids without shrinking upon cooling. Of course, in order that all moisture be driven from the fibreboard, the impregnating composition must be applied at a temperature higher than the boiling point of water, yet not so high as to burn or scorch the paperboard. I have found that a temperature of 325° F. is entirely satisfactory and safe, the flash point of my impregnating composition being over 400° F.

The objects of my invention are to provide an inexpensive water resistant and strength imparting impregnant 20 for corrugated paperboard, a process of making it and the paperboard made therewith.

Another object is to provide a paperboard impregnant that increases the column loading strength of corrugated paperboard to at least about 300 percent.

25 Still another object is to provide an impregnant which will stiffen the paperboard without imparting an extreme brittle condition.

A further object is to provide an impregnant for paperboard containers which will not contaminate or damage articles packaged therein.

A search for a satisfactory paperboard impregnant was made in which several inexpensive and water-proof materials were tested. Among the materials tested were:

- 35 (1) Paraffin.  
(2) A mixture of wood rosin and paraffin.  
(3) A mixture of wood rosin, paraffin and gilsonite.  
(4) Sulphur.

All of the materials would be satisfactory costwise in the highly competitive paperboard industry. Results of these comparative tests are shown below in Table I.

Table I

| Impregnating composition    | Pounds<br>Mate-<br>rial<br>Applied<br>per M<br>Sq. Ft. | Column Loading (percent)        |                                 |                                    | Beam Loading (percent)           |                                  |                                    |
|-----------------------------|--------------------------------------------------------|---------------------------------|---------------------------------|------------------------------------|----------------------------------|----------------------------------|------------------------------------|
|                             |                                                        | 50%<br>Rel.<br>Hum.,<br>72 hrs. | 99%<br>Rel.<br>Hum.,<br>72 hrs. | 24 hour<br>Water<br>Immer-<br>sion | 50%<br>Rel.<br>Hum.,<br>72 hours | 99%<br>Rel.<br>Hum.,<br>72 hours | 24 hour<br>Water<br>Immer-<br>sion |
|                             |                                                        |                                 |                                 |                                    |                                  |                                  |                                    |
| Untreated Board             |                                                        | 100                             | 61                              | 0                                  | 100                              | 50                               | 0                                  |
| 100% White Refined Paraffin | 105                                                    | 244                             | 163                             | 3                                  | 182                              | 118                              | 5                                  |
| 50% Limed Wood Rosin        |                                                        |                                 |                                 |                                    |                                  |                                  |                                    |
| 50% White Refined Paraffin  | 125                                                    | 341                             | 325                             | 47                                 | 223                              | 204                              | 41                                 |
| 50% Limed Wood Rosin        |                                                        |                                 |                                 |                                    |                                  |                                  |                                    |
| 40% White Refined Paraffin  | 141                                                    | 338                             | 322                             | 58                                 | 209                              | 182                              | 64                                 |
| 10% Gilsomite               |                                                        |                                 |                                 |                                    |                                  |                                  |                                    |
| 100% Sulphur                | 236                                                    | 354                             | 321                             | 30                                 | 232                              | 186                              | 32                                 |

NOTE.—Untreated board at 50% relative humidity equals 100%.

impregnated by immersing the corrugated paperboard into the impregnating composition in such a position so that the impregnating composition can flow freely through the flutes. The immersion time should be such that all bubbling and foaming ceases, indicating that all air and moisture has been driven from the paperboard. When the treated corrugated paperboard is removed from the vessel it must be supported so that all surplus impregnating composition can drain freely from the flutes and the paperboard surface as the corrugated paperboard will remain somewhat soft until the impregnating composition has cooled. Some care should be taken not to mash the flutes while draining.

I have found that surface deposits of the impregnating

Paraffin alone increases column loading strength about 2½ times and the material used per thousand square feet of paperboard is approximately 105 pounds. A mixture of 50 percent limed wood rosin and 50 percent paraffin on the other hand increases the column loading strength of corrugated paperboard approximately three and one-half times while using 125 pounds per thousand square feet of paperboard, furthermore the strength is not materially reduced at 99 percent relative humidity as in the case of 100 percent paraffin. When about 10 percent gilsonite is added to the limed wood rosin paraffin mixture, it further increases its strength at extreme wet conditions however, the addition of gilsonite does not increase the strength at other conditions and the ma-

terial required for one thousand square feet is substantially increased. Sulphur shows an increase of about three and one-half times but the material necessary to impregnate the paperboard amounts to 236 pounds per 5 square feet of paperboard. Furthermore, sulphur is unsatisfactory in that it is apt to be injurious to articles packaged therein such as commestables, etc.

Table I indicates that a mixture of limed wood rosin and paraffin will provide optimum results as an inexpensive paperboard impregnated. To determine at what ratio of paraffin to limed wood rosin best results could be obtained, further tests were conducted the results of which are as follows:

Table II.—Paraffin-limed wood rosin—formula variation

| Percent Paraffin | Percent Limed Wood Rosin | Lbs. impregnating composition Absorbed Per M Sq. Ft. | Column Loading—Ave. Max. Load in Lbs. |                    |
|------------------|--------------------------|------------------------------------------------------|---------------------------------------|--------------------|
|                  |                          |                                                      | 73° F., 50% R. H.                     | .90° F., 90% R. H. |
| 75               | 25                       | 90.7                                                 | 488                                   | 343                |
| 70               | 30                       | 96.5                                                 | 502                                   | 365                |
| 65               | 35                       | 99.7                                                 | 517                                   | 403                |
| 60               | 40                       | 102.8                                                | 562                                   | 424                |
| 55               | 45                       | 108.1                                                | 563                                   | 452                |
| 50               | 50                       | 116.9                                                | 601                                   | 451                |
| 45               | 55                       | 121.0                                                | 604                                   | 462                |
| 40               | 60                       | 127.4                                                | 623                                   | 520                |
| 35               | 65                       | 145.8                                                | 701                                   | 590                |
| 30               | 70                       | 160.5                                                | 707                                   | 586                |
| Plain Paperboard |                          | 173                                                  | 118                                   |                    |

It is readily seen from Table II that as the ratio of limed wood rosin to paraffin is increased, the column loading strength of corrugated paperboard likewise increases but at a progressively reduced rate while the quantity of impregnant absorbed per thousand square feet increases rapidly to an economically prohibitive amount. Furthermore at a ratio of limed wood rosin below 45% to limed wood rosin has a tendency to drop out of the mixture. A ratio of from 45 : 55 to 55 : 45 of paraffin to limed wood rosin respectively gives satisfactory column loading strength characteristics while not requiring excessive quantities of material per thousand square feet of paperboard.

Therefore, by way of illustration, and not by way of limitation the following specific formula has been found to produce excellent results:

Parts by weight  
White refined paraffin ..... 100  
Limed rosin (4.5%  $\text{Ca}(\text{OH})_2$ ) ..... 100

Heat to 325° F. with some occasional agitation to form a smooth homogeneous mixture.

It is understood that the embodiments herein described are illustrative and not restrictive, and it is also to be understood that the invention may be susceptible of embodiment in other modified forms, and that all such

modifications which are similar or equivalent hereto come equally within the scope of the claims next appearing.

What I claim is:

1. A water resistant and strength imparting impregnating composition for application to corrugated paperboard to increase the column loading strength thereof to at least about 300 percent; said composition consisting essentially of a homogeneous admixture of about 50% refined paraffin and about 50% limed rosin having about 4.5% lime content.

2. The process of compounding a homogeneous water resistant and strength imparting impregnating composition adapted for impregnating corrugated paperboard, said process comprising the following successive steps; charging about 500 pounds of refined paraffin and about 500 pounds of limed rosin having about 4.5% lime content into a suitable vessel and heating to about 325 degrees F., with some occasional mild agitation.

3. A corrugated paperboard sheet impregnated by immersion for at least about two minutes into a water resistant and strength imparting impregnating composition, said composition consisting essentially of a homogeneous admixture of about 50% refined paraffin and about 50% limed rosin having about 4.5% lime content, heated to about 325 degrees F.

4. A water resistant and strength imparting impregnating composition for application to corrugated paperboard to increase the column loading strength thereof to at least about 300%; said composition consisting essentially of a homogeneous admixture of refined paraffin and limed rosin having about 4.5% lime content, wherein the content of refined paraffin is within the range of from about 45 to 55 parts for each 100 parts by weight of the composition.

5. The process of compounding a homogeneous water resistant and strength imparting impregnating composition for impregnating corrugated paperboard, said process comprising the following successive steps: charging about 1,000 pounds of refined paraffin and limed rosin having about 4.5% lime content into a suitable vessel and heating to about 325° F. with some occasional mild agitation, wherein the content of refined paraffin is within the range of from about 450 to 550 pounds.

6. A corrugated paperboard sheet impregnated by immersion for at least about 2 minutes into a water resistant and strength imparting impregnating composition, said composition consisting essentially of a homogeneous admixture of refined paraffin and limed rosin having about 4.5% lime content, heated to about 325° F., wherein the content of refined paraffin is within the range of from about 45 to 55 parts to each 100 parts by weight of the composition.

References Cited in the file of this patent

UNITED STATES PATENTS

2,648,616 Gauthier ..... Aug. 11, 1953